# EUROPEAN PATENT SPECIFICATION

(11) **EP 3 330 016 B1**
(45) Date of publication and mention of the grant of the patent: **06.09.2023**
(21) Application number: 16830013.5
(22) Date of filing: 05.07.2016
(51) Int. Cl.: B21D 22/20, C23C 2/06, C23C 2/26, C23C 2/40, C25D 5/26, C25D 5/48, B21D 22/26, C21D 8/02, C21D 9/46

(54) **METHOD FOR PRODUCING HOT-PRESSED MEMBER**
VERFAHREN ZUR HERSTELLUNG EINES HEISSGEPRESSTEN ELEMENTS
PROCÉDÉ POUR LA PRODUCTION D'ÉLÉMENT FORMÉ À LA PRESSE À CHAUD

(30) Priority: 29.07.2015 JP 2015149092; 19.02.2016 JP 2016029871
(43) Date of publication of application: 06.06.2018
(73) Proprietor: JFE Steel Corporation, Tokyo 100-0011 (JP)
(72) Inventor: NAKAJIMA, Seiji, Tokyo 100-0011 (JP); ANDO, Satoru, Tokyo 100-0011 (JP)
(74) Representative: Grünecker Patent- und Rechtsanwälte PartG mbB
(86) International application number: PCT/JP2016/003196
(87) International publication number: WO 2017/017905

(56) References cited:
- EP-A1- 2 159 292
- EP-A1- 2 719 796
- WO-A1-2008/153183
- JP-A- 2014 014 834
- JP-A- 2015 071 810
- JP-A- 2015 071 810
- JP-A- 2015 094 006
- JP-A- 2015 104 753

## Description

### Technical Field

The present invention relates to a method for manufacturing a hot-pressed member which can preferably be used for, for example, chassis and body structure members of an automobile.

### Background Art

To date, for example, chassis and body structure members of an automobile have usually been manufactured by performing press working on steel sheets having a specified strength. Nowadays, since there is a strong demand for the weight reduction of an automobile body from the viewpoint of global environment conservation, efforts are being made to reduce the thickness of a steel sheet which is used for an automobile body by increasing the strength of the steel sheet. However, an increase in the strength of steel sheets causes a deterioration in press workability, and therefore there is an increase in the number of cases where it is difficult to form a steel sheet into desired shapes of the members.

In view of the situation described above, Patent Literature 1 proposes a working technique called hot pressing which makes it possible to realize an improvement in workability and an increase in strength at the same time by performing working and rapid cooling at the same time on a heated steel sheet by using a mold which is composed of a die and a punch. However, in the case of this hot pressing, since a steel sheet is heated to a high temperature of about 950°C before hot pressing is performed, scale (iron oxide) is generated on the surface of the steel sheet, and the flaking of the scale occurs when hot pressing is performed, which results in a problem in that a mold is damaged or the surface of a member is damaged after the hot pressing. Also, scale which remained on the surface of a member causes a deterioration in surface appearance and paint adhesiveness. Therefore, scale which is present on the surface of a member is usually removed by performing a treatment such as pickling or shot blasting. However, such a treatment makes a manufacturing process complex, and thus there is a decrease in productivity.

Moreover, for example, chassis and body structure members of an automobile are also required to have excellent corrosion resistance. However, since a hot-pressed member, which is manufactured by using the process described above, is not provided with an anti-corrosion film such as a coating layer, the member is very poor in terms of corrosion resistance.

Therefore, a hot-pressing technique is desired with which the generation of scale can be inhibited when heating is performed before hot pressing and with which the corrosion resistance of a hot-pressed member can be improved, and thus a steel sheet to be hot-pressed whose surface is coated with a film such as a coating layer and a method for hot pressing which utilizes the steel sheet have been proposed.

For example, Patent Literature 2 discloses a method for manufacturing a hot-pressed member excellent in terms of corrosion resistance whose surface is coated with a Zn-Fe-based compound or a Zn-Fe-Al-based compound by performing hot pressing on a steel sheet, which is coated with Zn or a Zn-based alloy.

In addition, Patent Literature 3 discloses a hot-pressed member excellent in terms of scale resistance, paint adhesiveness, after-painting corrosion resistance, and hydrogen entry resistance which is manufactured by forming a Ni diffusion region, a layer of an intermetallic compound, which is equivalent to the γ phase of a Zn-Ni alloy, and a ZnO layer in the surface layer of a steel sheet.

Moreover, Patent Literature 4 discloses a steel sheet to be hot-pressed which is manufactured by forming a ZnO layer, which inhibits the vaporization of Zn, in the surface layer of a Zn-based coating layer in advance, and indicates that it is possible to obtain a hot-pressed product having good surface appearance, excellent paint adhesiveness, and excellent after-painting corrosion resistance by using the steel sheet.
Further methods for manufacturing hot-pressed members are disclosed in JP 2015 071810 A and EP 2 159 292 A1.

### Citation List

### Patent Literature

PTL 1: UK Patent No. GB1490535
PTL 2: Japanese Patent No. 3663145
PTL 3: Japanese Patent No. 4849186
PTL 4: Japanese Patent No. 3582511

### Summary of Invention

### Technical Problem

As disclosed in the conventional techniques described above, using a zinc-based coated steel sheet as a steel sheet to be hot-pressed is effective for improving corrosion resistance. However, since the melting point of zinc is 419°C and the boiling point of zinc is 907°C, that is, since both are low, the melting of zinc in the coating layer and the vaporization of zinc from the coating layer occur in a heating process before hot pressing, which makes it difficult to stably manufacture a hot-pressed member having a homogeneous and good surface appearance.

For example, in the case of a hot-pressed member which is manufactured by using the method described in Patent Literature 2, since a zinc-coated steel sheet or a zinc-aluminum-coated steel sheet, whose coating layer has a low melting point, is used, the melting of the coating layer or the vaporization of zinc which occurs in a heating process before hot pressing is significant. As a result, a hot-pressed member, which is finally obtained, has, for example, a spotty inhomogeneous surface appearance or many white or black point-like defects. Therefore, it is difficult to obtain a hot-pressed member having a homogeneous and good surface appearance. Here, since not only a deterioration in surface appearance but also a deterioration in paint adhesiveness occur in a portion in which point-like defects exist, there is a strong demand for a technique for preventing point-like defects. However, an effective technique has not been proposed.

In the case of a hot-pressed member described in Patent Literature 3 which is manufactured by using a steel sheet coated with a Zn-Ni-alloy coating layer, which has a melting point higher than that of Zn, there is an improvement in the surface appearance of a hot-pressed member compared with the case where a zinc-coated steel sheet or a zinc-aluminum-coated steel sheet is used. However, it is not possible to completely prevent the generation of local point-like defects.

In the case where a steel sheet to be hot-pressed described in Patent Literature 4 is used, there is an improvement in the surface appearance of a hot-pressed member to some extent through the effect of a ZnO layer which is formed in the surface layer of the steel sheet. However, there is still a problem in that local point-like defects are generated in a portion in which the result of a treatment for forming a ZnO layer is inhomogeneous. In addition, there is a problem of a significant increase in cost when a treatment for forming a ZnO layer is performed, because it is necessary to use a method which involves, for example, an oxidizing treatment through the use of heat, a contact treatment with a solution, an electrolysis treatment in an aqueous solution, and a treatment of coating and drying a solution.

The present invention has been completed in order to solve the problems of the conventional techniques described above, and an object of the present invention is to provide a method for manufacturing a hot-pressed member excellent in terms of surface appearance with which it is possible to stably manufacture a hot-pressed member having a homogeneous and good surface appearance without causing a significant increase in cost.

### Solution to Problem

The present inventors, in order to solve the problems described above, diligently conducted investigations regarding a method for manufacturing a hot-pressed member excellent in terms of surface appearance. First, investigations regarding a state in which point-like defects are generated on the surface of a hot-pressed member were conducted. As a result, it was found that the position or number of point-like defects is not necessarily the same even if the same kind of zinc-based coated steel sheet is heated under the same condition. Also, it was found that it is not possible to completely prevent point-like defects even with a Zn-Ni-alloy-coated steel sheet, although a steel sheet coated with a Zn-Ni-alloy coating layer, which has a higher melting point than that of zinc-based coated steel sheet, can be used as a steel sheet to be hot-pressed more advantageously than a zinc-based coated steel sheet such as a galvanized steel sheet or a galvannealed steel sheet, which has a coating layer having a comparatively low melting point, from the viewpoint of inhibiting point-like defects from occurring.

From such facts, on the basis of the hypothesis that the generation of point-like defects depends not only on the kind of a coating layer and heating conditions but also on other factors such as a stain on the surface, verification experiments were conducted in which a zinc-based coated steel sheet was heated after the surface of the steel sheet had been stained or cleaned. As a result, it was found that point-like defects, which are generated on the surface of a hot-pressed member, are caused by stains due to, for example, dirt, dust, and fingerprint which are adhered to the surface of a coating layer. That is, it was found that there is a local increase in temperature due to extraneous matter derived from such stain materials being burned in a heating process before hot pressing work, which results in the vaporization of zinc being promoted due to the breakage of a ZnO layer with which the surface of the zinc-based coating layer has been covered, and which results in scale being generated in such a portion. In addition, it was further found that it is possible to significantly inhibit the generation of point-like defects by performing a surface-cleaning treatment in order to remove such stain materials before a heating process. Moreover, it was found that the effect of inhibiting point-like defects through the use of a surface-cleaning treatment before heating is realized not only in a process in which a zinc-based coated steel sheet is subjected to hot pressing work and cooling after having been heated but also in a process in which a zinc-based coated steel sheet is heated and cooled after having been subjected to cold pressing work, resulting in the completion of the present invention.

The method for manufacturing a hot-pressed member according to the present invention has been completed on the basis of such findings, and the subject matter of the present invention is as specified in the appended claims.

Here, in the present description, % used when describing the chemical composition of steel or a coating layer always means mass%.

### Advantageous Effects of Invention

According to the present invention, it is possible to stably manufacture a hot-pressed member having a homogeneous and good surface appearance without causing a significant increase in cost. The hot-pressed member which is manufactured by using the present invention can preferably be used for the chassis and body structure members of an automobile.

### Brief Description of Drawings

[Fig. 1] Fig. 1 is a diagram illustrating typical examples of the surface appearance of a hot-pressed member, where (a) is a photograph indicating a product having a good surface appearance and (b) is a photograph indicating a product having point-like defects.
[Fig. 2] Fig. 2 is a diagram illustrating typical examples of the surface appearance of point-like defects, where (a) is an enlarged photograph of a white defect and (b) is an enlarged photograph of a black defect.

### Description of Embodiments

### 1) Zinc-based coated steel sheet

In the method for manufacturing a hot-pressed member according to the present invention, a zinc-based coated steel sheet having a zinc-based coating layer on one or both sides thereof is used. Examples of a zinc-based coating layer include, but are not limited to, a galvanizing layer, a galvannealing layer, a hot-dip zinc-aluminum-alloy coating layer, a hot-dip zinc-aluminum-magnesium-alloy coating layer, a zinc electroplating layer, and a zinc-nickel-alloy electroplating layer, and all of the known zinc-based coating layers containing zinc may be used.

It is preferable that the coating weight on the surface of such a zinc-based coated steel sheet be 10 g/m² to 90 g/m² per side. In the case where the coating weight per side (hereinafter, also simply referred to as "coating weight") is 10 g/m² or more, the corrosion resistance does not become insufficient. On the other hand, in the case where the coating weight is 90 g/m² or less, there is no increase in cost. It is more preferable that the coating weight be 20 g/m² to 80 g/m². Here, it is possible to determine coating weight by using a wet analysis method. Specifically, for example, by dissolving the whole coating layer of a test piece whose coated area is known in an aqueous solution in which 1 g/L of hexamethylenetetramine is added as an inhibitor to a 6-mass%-hydrochloric acid aqueous solution, the coating weight of the coating layer should be derived from the amount of decrease in mass at this time.

It is preferable that the zinc-based coated steel sheet described above be a Zn-Ni-alloy-coated steel sheet having a coating layer on one or both sides thereof, in which the coating layer having a chemical composition containing 10 mass% to 25 mass% of Ni and the balance being Zn and inevitable impurities. In the case where the Ni content in the coating layer is 10 mass% to 25 mass%, since the structure of the coating layer becomes a γ phase structure, and since this γ phase has a high melting point of 881°C, there is an increase in the effect of inhibiting the generation of point-like defects to a higher level. Here a γ phase has one of the crystal structures of Ni₂Zn₁₁, NiZn₃, and Ni₅Zn₂₁, and it is possible to identify the structure by using an X-ray diffraction method. Here, an underlying coating layer such as a coating layer mainly containing, for example, Ni may be formed under the above-described coating layer.

### 2) Base steel sheet

In order to obtain the hot-pressed member according to the present invention, a hot-rolled steel sheet or a cold-rolled steel sheet having a chemical composition containing, by mass%, C: 0.15% to 0.50%, Si: 0.05% to 2.00%, Mn: 0.5% to 3.0%, P: 0.10% or less, S: 0.05% or less, Al: 0.10% or less, N: 0.010% or less, and the balance being Fe and inevitable impurities may be used as a base steel sheet for a zinc-based coating layer. In the case where a hot-rolled steel sheet or a cold-rolled steel sheet having such a chemical composition is used as a base steel sheet, it is possible to obtain a hot-pressed member having a desired high strength of, for example, 980 MPa or more.

The reasons for the limitations on the constituent chemical elements will be described hereafter.

### C: 0.15% to 0.50%

C is a chemical element which increases the strength of steel, and it is necessary that the C content be 0.15% or more in order to control the tensile strength (hereinafter, also referred to as "TS") of a hot-pressed member to be 980 MPa or more. On the other hand, in the case where the C content is more than 0.50%, there is a significant deterioration in the blanking performance of a steel sheet as a material. Therefore, it is preferable that the C content be 0.15% to 0.50%.

### Si: 0.05% to 2.00%

Si is, like C, a chemical element which increases the strength of steel, and it is necessary that the Si content be 0.05% or more in order to control the TS of a hot-pressed member to be 980 MPa or more. On the other hand, in the case where the Si content is more than 2.00%, there is a significant increase in the amount of a surface defect, which is called red scale, generated when hot rolling is performed, there is an increase in rolling load, and there is a deterioration in the ductility of a hot-rolled steel sheet. Moreover, in the case where the Si content is more than 2.00%, there may be a negative effect on coatability when a coating treatment is performed in order to form a coating film containing mainly Zn and Al on the surface of a steel sheet. Therefore, it is preferable that the Si content be 0.05% to 2.00%.

### Mn: 0.5% to 3.0%

Mn is a chemical element which is effective for improving hardenability by inhibiting ferrite transformation and which is effective for decreasing a heating temperature before hot pressing is performed, because Mn decreases the Ac₃ transformation temperature. It is necessary that the Mn content be 0.5% or more in order to realize such effects. On the other hand, in the case where the Mn content is more than 3.0%, since Mn is segregated, there is a deterioration in the homogeneity of the properties of a steel sheet as a material and a hot-pressed member. Therefore, it is preferable that the Mn content be 0.5% to 3.0%.

### P: 0.10% or less

In the case where the P content is more than 0.10%, since P is segregated, there is a deterioration in the homogeneity of the properties of a steel sheet as a material and a hot-pressed member, and there is a significant decrease in toughness. Therefore, it is preferable that the P content be 0.10% or less.

### S: 0.05% or less

In the case where the S content is more than 0.05%, there is a decrease in the toughness of a hot-pressed member. Therefore, it is preferable that the S content be 0.05% or less.

### Al: 0.10% or less

In the case where the Al content is more than 0.10%, there is a deterioration in the blanking performance and hardenability of a steel sheet as a material. Therefore, it is preferable that the Al content be 0.10% or less.

### N: 0.010% or less

In the case where the N content is more than 0.010%, since nitrides of AlN are formed when hot rolling is performed or when heating is performed before hot pressing work is performed, there is a deterioration in the blanking performance and hardenability of a steel sheet as a material. Therefore, it is preferable that the N content be 0.010% or less.

The remainder is Fe and inevitable impurities. Moreover, it is preferable that at least one selected from Cr: 0.01% to 1.0%, Ti: 0.01% to 0.20%, and B: 0.0005% to 0.0800% and Sb: 0.003% to 0.030% be added separately or at the same time in addition to the chemical composition described above for the reasons described below.

### Cr: 0.01% to 1.0%

Cr is a chemical element which is effective for increasing the strength of steel and improving hardenability of steel. It is preferable that the Cr content be 0.01% or more in order to realize such effects. On the other hand, in the case where the Cr content is more than 1.0%, there is a significant increase in cost. Therefore, it is preferable that the upper limit of the Cr content be 1.0%.

### Ti: 0.01% to 0.20%

Ti is a chemical element which is effective for increasing the strength of steel and which is effective for increasing toughness by decreasing a crystal grain size. In addition, Ti is a chemical element which is effective for realizing the effect of improving hardenability through the use of solid solution B by forming nitrides more readily than B, which will be described below. Therefore, it is preferable that the Ti content be 0.01% or more. However, in the case where the Ti content is more than 0.20%, there is a significant increase in rolling load when hot rolling is performed, and there is a decrease in the toughness of a hot-pressed member. Therefore, it is preferable that the upper limit of the Ti content be 0.20%.

### B: 0.0005% to 0.0800%

B is a chemical element which is effective for improving hardenability when hot pressing is performed and for increasing toughness after the hot pressing. It is preferable that the B content be 0.0005% or more in order to realize such effects. On the other hand, in the case where the B content is more than 0.0800%, there is a significant increase in rolling load when hot rolling is performed, and, for example, cracking occurs in a steel sheet due to the formation of a martensite phase and a bainite phase after the hot rolling. Therefore, it is preferable that the upper limit of the B content be 0.0800%.

### Sb: 0.003% to 0.030%

Sb is effective for inhibiting the formation of a decarburized layer in the surface layer of a steel sheet in a process in which a zinc-based coated steel sheet is subjected to heating followed by hot pressing work and cooling. It is necessary that the Sb content be 0.003% or more in order to realize such an effect. On the other hand, in the case where the Sb content is more than 0.030%, since there is an increase in rolling load, there is a decrease in productivity. Therefore, it is preferable that the Sb content be 0.003% to 0.030%.

### 3) Hot pressing process

In the method for manufacturing a hot-pressed member according to the present invention, a hot-pressed member is manufactured by using one of the processes in the two embodiments described below as a hot pressing process.

The first embodiment is a method for manufacturing a hot-pressed member and is a hot pressing process called direct process in which a zinc-based coated steel sheet is subjected to heating to a temperature range from the Ac3 transformation temperature to 1000°C followed by hot pressing work and cooling. In the case where the heating temperature is lower than the Ac3 transformation temperature, since there is an insufficient degree of quenching of a steel sheet, there may be a case where it is not possible to achieve the desired strength. In addition, in the case where the heating temperature is higher than 1000°C, there is an economic disadvantage from the viewpoint of energy, and it is difficult to manufacture a hot-pressed member having a homogeneous and good surface appearance due to the significant generation of point-like defects. In addition, cooling after hot pressing work may be performed by using a mold at the same time as hot pressing work, or the cooling may be performed by using a coolant such as water at the same time as hot pressing work or immediately after the hot pressing work.

The second embodiment is a method for manufacturing a hot-pressed member and is a hot pressing process called indirect process in which a zinc-based coated steel sheet is subjected to cold pressing work followed by heating to a temperature range from the Ac3 transformation temperature to 1000°C and cooling. In this process, cold pressing work is first performed before a zinc-based coated steel sheet is heated. Subsequently, the cold-pressed member is subjected to heating followed by cooling. The heating temperature is set to be in a temperature range from the Ac3 transformation temperature to 1000°C for the reasons described above. Cooling may be performed by using a mold which is used for cooling a member or by using a coolant such as water. In addition, when cooling is performed by using a mold, work may be added by performing hot pressing.

Here, the term "heating temperature" means the maximum end-point temperature of a steel sheet. In addition, examples of a method for performing the heating described above include heating which utilizes, for example, an electric furnace or a gas furnace, direct-fired heating, electrical heating, high-frequency heating, and induction heating.

### 4) Surface-cleaning treatment

In the method for manufacturing a hot-pressed member according to the present invention, a surface-cleaning treatment is performed on a zinc-based coated steel sheet before the zinc-based coated steel sheet is heated in order to remove stains due to, for example, dirt, dust, and fingerprint which are adhered to the surface of a coating layer. This surface-cleaning treatment is an important requirement in the present invention. In the case where this surface-cleaning treatment is not performed, point-like defects are generated as illustrated in Fig. 1(b). On the other hand, in the case where a surface-cleaning treatment is performed, it is possible to manufacture a product having a good surface appearance as illustrated in Fig. 1(a). Here, examples of point-like defects include a white defect illustrated in Fig. 2(a), which is a mark of intense vaporization of zinc left at the position of the breakage of a ZnO layer, with which the surface of a zinc-based coating layer has been covered, and a black defect illustrated in Fig. 2(b), which is generated as a result of scale being generated through the progress of the oxidation of a base steel sheet at the position of a white defect. Since, both of the point-like defects deteriorate surface appearance and paint adhesiveness, it is necessary to inhibit point-like defects as much as possible by performing a surface-cleaning treatment. As described above, a surface-cleaning treatment according to the present invention is a treatment which removes the origins of point-like defects.

It is necessary to perform a surface-cleaning treatment before a heating process. Therefore, in the case of the first embodiment described above (in which a zinc-based coated steel sheet is subjected to heating to a temperature range from the Ac3 transformation temperature to 1000°C followed by hot pressing work), it is necessary to perform a surface-cleaning treatment on a steel sheet in the form of a coiled steel sheet or in the form of a cut steel sheet or a steel sheet blank, which has been cut out of the coiled steel sheet. In addition, in the case of the second embodiment described above (in which a zinc-based coated steel sheet is subjected to cold pressing work followed by heating to a temperature range from the Ac3 transformation temperature to 1000°C), a surface-cleaning treatment may be performed on a steel sheet in the form of a coiled steel sheet or in the form of a cut steel sheet or a steel sheet blank, which has been cut out of the coiled steel sheet, or on a cold-pressed member after cold pressing work. Here, in any one of the first embodiment and the second embodiment, it is preferable that the period of time from the end of a surface-cleaning treatment to the beginning of heating be as short as possible. In addition, it is preferable that a surface-cleaning treatment be performed on a steel sheet in the form of a steel sheet blank, because this facilitates the treatment with a high level of surface cleaning effect.

In the case alkaline degreasing is performed as a surface-cleaning treatment by using an alkaline degreasing liquid having a pH of 12.5 or more, since there is an excessive effect of dissolving a zinc-based coating layer, the generation of point-like defects is conversely promoted due to inhomogeneous dissolution, and there is a deterioration in corrosion resistance due to a decrease in coating weight. Therefore, according to the invention, alkaline degreasing is performed as a surface-cleaning treatment by using an alkaline degreasing liquid, the pH of the alkaline degreasing liquid is set to be less than 12.5. Moreover, it is preferable that the process of a surface-cleaning treatment have a low cost. In the case where apparatuses for cold pressing work has an apparatus for performing the combination of wash-oil application and brushing, such equipment can preferably be used for hot pressing work, because it is possible to perform a treatment at low cost with a high cleaning effect by using such equipment.

### EXAMPLES

A cold-rolled steel sheet having a chemical composition containing, by mass%, C: 0.23%, Si: 0.25%, Mn: 1.2%, P: 0.01%, S: 0.01%, Al: 0.03%, N: 0.005%, Cr: 0.2%, Ti: 0.02%, B: 0.0022%, Sb: 0.008%, and the balance being Fe and inevitable impurities, an Ac3 transformation temperature of 820°C, and a thickness of 1.6 mm was used as a base steel sheet. The surface of this cold-rolled steel sheet was coated with one of a galvanizing layer, a hot-dip Zn-Al-alloy coating layer (Al content: 55 mass%), a galvannealing layer (Fe content: 10 mass%), a Zn electroplating layer, and a Zn-Ni-alloy electroplating layer (Ni content: 12 mass%) and cut into a sample having a size of 200 mm × 300 mm.

The sample obtained as described above was subjected to a surface-cleaning treatment. A surface-cleaning treatment was performed by using one of A: a wiping method with waste cloth, B: a brushing method, C: a combined method of wash-oil application and brushing, D: an alkaline degreasing method (pH: 12.0), and E: a solvent degreasing method. As comparative examples, samples which had been subjected to F: strong alkaline degreasing (pH: 13.0) and samples which had not been subjected to a surface-cleaning treatment were also prepared.

Wiping with waste cloth was performed by using waste cloth (Cleaning White Stockinet Waste (Cotton) produced by Nihon Waste Co., Ltd.) and by wiping the surface of a sample twice with a reciprocating movement of a hand.

Brushing was performed by using a nylon-fiber plant brush (SK-type Straight Brush produced by Showa Kogyo Co., Ltd.) and by brushing the surface of a sample twice with a reciprocating movement of a hand.

The combination of wash-oil application and brushing was performed by performing brushing as described above after having applied a wash rust-prevention oil (PRETON R352L produced by Sugimura Chemical Industrial Co., Ltd.) to the surface of a sample so that the amount of oil applied was 2.0 g/m².

Alkaline degreasing was performed by spraying a sample with an alkaline degreasing liquid (CL-N364S, 20g/L, 60°C, produced by Nihon Parkerizing Co., LTD.) for 10 seconds, and thereafter performing water washing followed by drying. Here, at this time, the pH of the alkaline degreasing liquid was 12.0.

Solvent degreasing was performed by immersing a sample in a combined solvent of toluene and ethanol having a mixture ratio of 1:1, and thereafter performing ultrasonic cleaning for one minute and drying.

Strong alkaline degreasing, which was performed as a comparative example, was performed by immersing a sample in a strong alkaline degreasing liquid (NaOH aqueous solution, pH: controlled to be 13.0, 50°C) for 5 seconds, and thereafter performing water washing followed by drying.

Subsequently, the sample was heated in an electric furnace at a temperature of 950°C so that duration of the sample in the electric furnace was 8 minutes, the sample was taken out of the furnace immediately after completion of heating, and then held in a flat mold made of Al in order to perform a rapid cooling treatment (cooling rate: 50°C/s).

The surface appearance of the samples (zinc-based coated steel sheets) obtained as described above was evaluated by using the following method.

Ten samples were each prepared under the same condition in order to increase the judgment accuracy of surface appearance. After having performed a visual test regarding the state of point-like defects of the samples, surface appearance was judged on the basis of the judgment criteria below, and the case of ⊙ or O was judged as satisfactory. Here, in the examples of the present invention, although the effect of the present invention was evaluated on the basis of the evaluation of the surface appearance after having heated and cooled a flat sheet as described above without performing practical press forming which utilized a direct process or an indirect process, the results of the present evaluation are the same as those of the evaluation of the surface appearance after having performed practical press forming which utilizes the above-mentioned two processes, because the surface appearance after having performed heating and cooling depends on whether or not stain components exist on the surface of the sample and on the effect of removing the stain components.
⊙: 10 out of the 10 samples had no point-like defect
O: 8 to 9 out of the 10 samples had no point-like defect
Δ: 5 to 7 out of the 10 samples had no point-like defect
×: 0 to 4 out of the 10 samples had no point-like defect

The results of the evaluation of surface appearance are given in Table 1 in combination with the manufacturing conditions.

**[Table 1]**

| Steel Shee t No. | Coating Layer | | Surface-cleaning Treatment | | Surface Appearance | Note |
|---|---|---|---|---|---|---|
| | Type * | Coating Weight per Side (g/m²) | Code | Treatment Method | | |
| 1 | Gl | 60 | A | Wiping with Waste Cloth | O | Reference Example |
| 2 | GL | 80 | A | Wiping with Waste Cloth | O | Reference Example |
| 3 | GA | 20 | A | Wiping with Waste Cloth | O | Reference Example |
| 4 | GA | 45 | A | Wiping with Waste Cloth | O | Reference Example |
| 5 | GA | 90 | A | Wiping with Waste Cloth | O | Reference Example |
| 6 | EG | 40 | A | Wiping with Waste Cloth | O | Reference Example |
| 7 | ZN | 10 | A | Wiping with Waste Cloth | ⊙ | Reference Example |
| 8 | ZN | 60 | A | Wiping with Waste Cloth | ⊙ | Reference Example |
| 9 | ZN | 90 | A | Wiping with Waste Cloth | ⊙ | Reference Example |
| 10 | GI | 60 | B | Brushing | O | Reference Example |
| 11 | GL | 80 | B | Brushing | O | Reference Example |
| 12 | GA | 20 | B | Brushing | O | Reference Example |
| 13 | GA | 45 | B | Brushing | O | Reference Example |
| 14 | GA | 90 | B | Brushing | O | Reference Example |
| 15 | EG | 40 | B | Brushing | O | Reference Example |
| 16 | ZN | 10 | B | Brushing | ⊙ | Reference Example |
| 17 | ZN | 60 | B | Brushing | ⊙ | Reference Example |
| 18 | ZN | 90 | B | Brushing | ⊙ | Reference Example |
| 19 | GI | 60 | C | Wash-oil Application + Brushing | ⊙ | Reference Example |
| 20 | GL | 80 | C | Wash-oil Application + Brushing | ⊙ | Reference Example |
| 21 | GA | 20 | C | Wash-oil Application + Brushing | ⊙ | Reference Example |
| 22 | GA | 45 | C | Wash-oil Application + Brushing | ⊙ | Reference Example |
| 23 | GA | 90 | C | Wash-oil Application + Brushing | ⊙ | Reference Example |
| 24 | EG | 40 | C | Wash-oil Application + Brushing | ⊙ | Reference Example |
| 25 | ZN | 10 | C | Wash-oil Application + Brushing | ⊙ | Reference Example |
| 26 | ZN | 60 | C | Wash-oil Application + Brushing | ⊙ | Reference Example |
| 27 | ZN | 90 | C | Wash-oil Application + Brushing | ⊙ | Reference Example |
| 28 | GI | 60 | D | Alkaline Degreasinq | ⊙ | Example |
| 29 | GL | 80 | D | Alkaline Degreasing | ⊙ | Example |
| 30 | GA | 20 | D | Alkaline Degreasing | ⊙ | Example |
| 31 | GA | 45 | D | Alkaline Degreasing | ⊙ | Example |
| 32 | GA | 90 | D | Alkaline Degreasing | ⊙ | Example |
| 33 | EG | 40 | D | Alkaline Degreasing | ⊙ | Example |
| 34 | ZN | 10 | D | Alkaline Degreasing | ⊙ | Example |
| 35 | ZN | 60 | D | Alkaline Degreasing | O | Example |
| 36 | ZN | 90 | D | Alkaline Degreasing | O | Example |
| 37 | GI | 60 | E | Solvent Degreasing | ⊙ | Reference Example |
| 38 | GL | 80 | E | Solvent Degreasing | ⊙ | Reference Example |
| 39 | GA | 20 | E | Solvent Degreasing | ⊙ | Reference Example |
| 40 | GA | 45 | E | Solvent Degreasing | ⊙ | Reference Example |
| 41 | GA | 90 | E | Solvent Degreasing | ⊙ | Reference Example |
| 42 | EG | 40 | E | Solvent Degreasing | ⊙ | Reference Example |
| 43 | ZN | 10 | E | Solvent Degreasing | ⊙ | Reference Example |
| 44 | ZN | 60 | E | Solvent Degreasing | ⊙ | Reference Example |
| 45 | ZN | 90 | E | Solvent Degreasing | ⊙ | Reference Example |
| 46 | GI | 60 | F | Strong Alkaline Deqreasing | × | Comparative Example |
| 47 | GL | 80 | F | Strong Alkaline Degreasing | × | Comparative Example |
| 48 | GA | 20 | F | Strong Alkaline Degreasing | × | Comparative Example |
| 49 | GA | 45 | F | Strong Alkaline Degreasing | × | Comparative Example |
| 50 | GA | 90 | F | Strong Alkaline Degreasing | × | Comparative Example |
| 51 | EG | 40 | F | Strong Alkaline Degreasing | × | Comparative Example |
| 52 | ZN | 10 | F | Strong Alkaline Degreasing | Δ | Comparative Example |
| 53 | ZN | 60 | F | Strong Alkaline Degreasing | Δ | Comparative Example |
| 54 | ZN | 90 | F | Strong Alkaline Degreasing | Δ | Comparative Example |
| 55 | GI | 60 | - | No Treatment | × | Comparative Example |
| 56 | GL | 80 | - | No Treatment | × | Comparative Example |
| 57 | GA | 20 | - | No Treatment | × | Comparative Example |
| 58 | GA | 45 | - | No Treatment | × | Comparative Example |
| 59 | GA | 90 | - | No Treatment | × | Comparative Example |
| 60 | EG | 40 | - | No Treatment | × | Comparative Example |
| 61 | ZN | 10 | - | No Treatment | Δ | Comparative Example |
| 62 | ZN | 60 | - | No Treatment | Δ | Comparative Example |
| 63 | ZN | 90 | - | No Treatment | Δ | Comparative Example |

| | | | | | | |
|---|---|---|---|---|---|---|
| * GI: galvanizing layer GL: hot-dip Zn-AI-alloy coating layer (Al content: 55 mass%) GA: galvannealing layer (Fe content: 10 mass%) EG: Zn electroplating layer ZN: Zn-Ni-alloy electroplating layer (Ni content: 12 mass%) | | | | | | |

It is clarified that all the zinc-based coated steel sheets (examples of the present invention), which were manufactured by performing a surface-cleaning treatment in the manufacturing method according to the present invention, were excellent in terms of surface appearance. In particular, it is clarified that the surface appearance was absolutely excellent in the case where a Zn-Ni-alloy-electroplated steel sheet was used. On the other hand, the zinc-based coated steel sheet (comparative example), which was subjected to degreasing with a strong alkali having a pH of 12.5 or more, and the zinc-based coated steel sheet (comparative example), which was not subjected to a surface-cleaning treatment, were poor in terms of surface appearance.

## Claims

1. A method for manufacturing a hot-pressed member having an excellent surface appearance, the method comprising heating a zinc-based coated steel sheet to a temperature range from the Ac3 transformation temperature to 1000°C, performing hot pressing work, and performing cooling, wherein a surface-cleaning treatment is performed on the zinc-based coated steel sheet before the heating is performed, and wherein the surface-cleaning treatment is performed using alkaline degreasing at pH of less than 12.5.

2. A method for manufacturing a hot-pressed member having an excellent surface appearance, the method comprising performing cold pressing work on a zinc-based coated steel sheet, heating the zinc-based coated steel sheet to a temperature range from the Ac3 transformation temperature to 1000°C, and cooling the heated steel sheet, wherein a surface-cleaning treatment is performed on the zinc-based coated steel sheet before the heating is performed, and wherein the surface-cleaning treatment is performed using alkaline degreasing at pH of less than 12.5.

3. The method for manufacturing a hot-pressed member according to Claim 1 or 2, wherein the zinc-based coated steel sheet is a Zn-Ni-alloy-coated steel sheet having a coating layer on one or both sides of the Zn-Ni-alloy-coated steel sheet, and the coating layer has a chemical composition containing 10 mass% to 25 mass% of Ni and the balance being Zn and inevitable impurities and a coating weight per side of 10 g/m² to 90 g/m².

## Patentansprüche

1. Verfahren zum Herstellen eines Heißpressteils mit einem hervorragenden Oberflächenerscheinungsbild, wobei das Verfahren das Erhitzen eines zinkbasierten beschichteten Stahlblechs zu einem Temperaturbereich von der Ac3-Übergangstemperatur zu 1000°C, das Durchführen einer Heißpressarbeit und das Durchführen eines Kühlens umfasst, wobei eine Oberflächenreinigungsbehandlung auf dem zinkbasierten beschichteten Stahlblech durchgeführt wird, bevor das Erhitzen durchgeführt wird, und wobei die Oberflächenreinigungsbehandlung unter Verwendung einer alkalischen Entfettung bei einem pH-Wert von weniger als 12,5 durchgeführt wird.

2. Verfahren zum Herstellen eines Heißpressteils mit einem hervorragenden Oberflächenerscheinungsbild, wobei das Verfahren das Durchführen einer Kaltpressarbeit auf einem zinkbasierten beschichteten Stahlblech, das Erhitzen des zinkbasierten beschichteten Stahlblechs zu einem Temperaturbereich von der Ac3-Übergangstemperatur zu 1000°C und das Kühlen des erhitzen Stahlblechs umfasst, wobei eine Oberflächenreinigungsbehandlung auf dem zinkbasierten beschichteten Stahlblech durchgeführt wird, bevor das Erhitzen durchgeführt wird, und wobei die Oberflächenreinigungsbehandlung unter Verwendung einer alkalischen Entfettung bei einem pH-Wert von weniger als 12,5 durchgeführt wird.

3. Verfahren zum Herstellen eines Heißpressteils nach Anspruch 1 oder 2, wobei das zinkbasierte beschichtete Stahlblech ein Zn-Ni-Legierung-beschichtetes Stahlblech ist, das eine Beschichtungsschicht auf einer oder beiden Seiten des Zn-Ni-Legierung-beschichteten Stahlblechs aufweist, wobei die Beschichtungsschicht eine chemische Zusammensetzung, die 10 Massenprozent bis 25 Massenprozent Ni und ansonsten Zn und unvermeidliche Verunreinigungen enthält, und ein Beschichtungsgewicht pro Seite von 10 g/m² bis 90 g/m² aufweist.

## Revendications

1. Procédé de fabrication d'un élément pressé à chaud ayant un excellent aspect de surface, le procédé comprenant le chauffage d'une tôle d'acier revêtue à base de zinc à une plage de température allant de la température de transformation Ac3 à 1000°C, la réalisation d'un travail de pressage à chaud et la réalisation d'un refroidissement, dans lequel un traitement de nettoyage de surface est réalisé sur la tôle d'acier revêtue à base de zinc avant la réalisation du chauffage, et dans lequel le traitement de nettoyage de surface est réalisé en utilisant un dégraissage alcalin à un pH inférieur à 12,5.

2. Procédé de fabrication d'un élément pressé à chaud ayant un excellent aspect de surface, le procédé comprenant la réalisation d'un travail de pressage à froid sur une tôle d'acier revêtue à base de zinc, le chauffage de la tôle d'acier revêtue à base de zinc à une plage de température allant de la température de transformation Ac3 à 1000°C, et le refroidissement de la tôle d'acier chauffée, dans lequel un traitement de nettoyage de surface est réalisé sur la tôle d'acier revêtue à base de zinc avant la réalisation du chauffage, et dans lequel le traitement de nettoyage de surface est réalisé en utilisant un dégraissage alcalin à un pH inférieur à 12,5.

3. Procédé de fabrication d'un élément pressé à chaud selon la revendication 1 ou 2, dans lequel la tôle d'acier revêtue à base de zinc est une tôle d'acier revêtue d'un alliage Zn-Ni ayant une couche de revêtement sur un ou deux côtés de la tôle d'acier revêtue d'un alliage Zn-Ni, et la couche de revêtement a une composition chimique contenant 10% en masse à 25% en masse de Ni et le reste étant du Zn et des impuretés inévitables et un poids de revêtement par côté de 10 g/m² à 90 g/m².
